

# UNITED STATES PATENT OFFICE.

HIRAM Y. McBRIDE, OF ARTESIA, NEW MEXICO, ASSIGNOR TO THE UNITED STATES WOOL COMPANY, OF DENVER, COLORADO, A CORPORATION OF ARIZONA.

## PROCESS OF TREATING WOOL.

1,323,641.

Specification of Letters Patent.

Patented Dec. 2, 1919.

No Drawing.

Application filed January 15, 1917. Serial No. 142,470.

To all whom it may concern:

Be it known that I, HIRAM Y. McBRIDE, a citizen of the United States, residing at Artesia, New Mexico, have invented a certain new and useful Process of Treating Wool, of which the following is a specification.

The invention consists in a new and improved process of preparing raw wool for utilization by the consumer in spinning, weaving, etc.

The term "wool" as herein used comprises the hair of various animals, such as sheep, goats, or other animals whose hair may be utilized for spinning or weaving, or in other arts. Sheep wool will be mentioned as a particular example, but the conditions pertaining to this wool exist in all wool when clipped, to a greater or less degree.

Raw wool, that is wool as clipped from the animal, is usually tangled, knotted or matted and contains grease, suint, manure, dirt, and vegetable matter such as burs, twigs, etc.

The commercial method of cleaning wool has been a wet process, resulting in the production of a large amount of greasy and offensive cleaning fluid which has usually been discharged into streams or into waste pools. In addition to the obnoxious features of this disposition of waste material, the wet process is more or less inefficient; the cleaning material employed more or less injures the wool and no adequate provision is made for combing, separating or straightening the wool incident to cleaning it.

For the objectionable wet process I substitute a mode of treating the wool with dry material, and in connection with this cleaning I provide for combing, separating or straightening the wool so that the final product is extremely clean, straight and free from knots or matted portions. The process does not in any respect injure the wool fiber and the discharged cleaning material carrying the grease, suint and dirt with it is a substantially dry solid of inoffensive character and may be stored without creating objectionable conditions.

The process in one form consists in separating or combing the wool in the presence of a suitable dry cleaning material. This material is usually a finely divided substance having as one important characteristic great grease-absorbing capacity. A very effective,

and preferred material, is suitably treated gypsum or calcium sulfate. Preferably, this gypsum is heated to drive off practically all of its water and is pulverized more or less, the finer pulverizing being desirable since very fine material affords an increased contact surface for cleaning purposes and is, therefore, most effective.

Instead of hydrated gypsum, treated as above, originally anhydrous gypsum suitably pulverized may be used.

The cleaning powder is applied to the wool in the process of combing, which is usually performed in suitable machines having toothed or spiked members to pull, straighten, separate and comb the wool fiber, and very quickly loosens and absorbs the grease and suint and moisture, and releases the other foreign material which is then easily discharged from the wool along with the cleaning powder. Provision is usually made in the combing machines for discharging dirt at suitable places, as for instance, by providing screened bottoms in the combing machines, or in arranging for discharge of the powder and dirt at intermediate points as the wool passes from one unit of the machine to another.

Cleaning material may be applied at one or more points in the progression of the wool through the combing devices, depending on conditions.

A refinement of the process which is desirable in some cases consists in a particular way of handling the cleaning material, namely in taking the cleaning powder discharged from the wool with its contained greases and dirt at a relatively late stage in the cleaning operation and transferring this material to the cleaning apparatus at a relatively earlier stage in the cleaning operation. As the wool progresses, it, of course, becomes relatively cleaner and the powder applied at a later stage in the process extracts relatively less foreign matter from the wool. This powder is therefore still relatively clean and may be used over again in an earlier stage of the process to extract a substantial part of the foreign matter from the relatively dirtier wool. In a complete development of this feature of the invention perfectly clean powder will be applied to the wool at its last cleaning stage; this powder will absorb very little extraneous matter; the powder is then taken to an in-

termediate point in the cleaning operation and put through the wool again, and in this step it absorbs a substantial amount of extraneous matter and the powder becomes correspondingly soiled or impregnated with greases and dirt, and this relatively dirty powder may then be put through the wool again at the earliest cleaning stage, where it absorbs extraneous matter up to its absorption capacity. The powder is then fully impregnated with greases and dirt and is stored or treated to recover valuable constituents or otherwise disposed of. The disposition of the powder after performing its cleaning function does not constitute a part of this invention.

A further feature of the invention consists in applying the cleaning material to the wool in storage or receiving bins as the raw wool is received from various sources, or in applying the material to the wool on sorting or feeding tables adjacent to the combing machine. This preliminary application of cleaning material causes the separation of a large part of the dirt before the combing or separating process commences, and thus the operation of combing is facilitated and the machines are relieved of the necessity of disposing of a large part of the waste material. The application of the cleaning medium to the wool for an indefinite period has no injurious effect on the wool so far as can be determined and, on the contrary, the effect of the cleaning medium is only beneficial. A further feature of the process consists in applying to the wool at a suitable point in the process a pulverized dry softening or lubricating material, such as talcum. In one form of the invention, the talcum is applied to the wool after most or all of the cleaning material and extraneous matter have been discharged from the wool. This application serves to soften and lubricate the fibers and to facilitate the final combing, which may be performed after application of the lubricant, and also serves to some extent to bleach the wool. A variation of the process consists in applying more or less of the talcum or other similar lubricant in conjunction with the cleaning material in a suitable proportion at some point in the combing operation. As a last step in the process, the cleaning material or the talcum, or both, are beaten out or otherwise removed from the wool, which is left in a beautifully soft, clean and straight condition, free from animal grease and suint and free from odor, and also un-

affected by the cleaning process as to any of its characteristics which are valuable in the arts.

Such material as suitably treated gypsum has been found to have remarkable capacity to attack and remove animal grease and suint, and in doing so to effectively remove other foreign material from the wool with a great reduction in the necessary manipulation of the wool. Whether the cleaning effect of the gypsum involves any intermediate chemical reactions, or whether the effect is purely physical, is difficult to determine, but whatever the action may be there is no evidence in the process of any injurious reactions and the most careful inspection of the completed product fails to show any injury to the wool whatsoever, as above stated.

Although suitably treated gypsum is the best cleaning agent I have discovered, other materials having a similar or equivalent effect may be used in some cases. Pulverized talcum is also the best lubricating and softening agent I have discovered up to this time, but other materials having similar or equivalent characteristics in respect to lubricating or softening the wool fiber, etc., may be substituted in some cases.

I claim:

1. The process of cleaning wool, consisting in applying pulverized dry cleaning material to wool to preliminarily remove a large part of the extraneous matter therefrom and then combing the wool in the presence of similar cleaning material to separate and straighten the wool and at the same time remove the remaining extraneous matter.

2. The process of cleaning wool, consisting in combing and cleaning wool and thereafter applying a pulverized dry lubricating material to the wool.

3. The process of cleaning wool, consisting in combing the wool in the presence of a pulverized dry cleaning material and a suitable proportion of a pulverized dry lubricating material.

4. The process of cleaning wool consisting in combing wool in the presence of pulverized dry cleaning material in progressive stages and transferring the cleaning material from a relatively late cleaning stage to the wool at relatively earlier cleaning stage to utilize the full absorptive capacity of the material.

HIRAM Y. McBRIDE.